

Apr. 3, 1923

1,450,704

J. A. SINGMASTER ET AL

PRODUCTION OF ZINC OXIDE

Filed Feb. 18, 1920



Inventors  
James A. Singmaster  
Frank G. Breyer  
By their Attorneys  
Pennie, Davis, Marren & Edmonds

## UNITED STATES PATENT OFFICE.

JAMES A. SINGMASTER AND FRANK G. BREYER, OF PALMERTON, PENNSYLVANIA,  
ASSIGNORS TO NEW JERSEY ZINC COMPANY, OF NEW YORK, N. Y., A CORPORATION  
OF NEW JERSEY.

## PRODUCTION OF ZINC OXIDE

Application filed February 18, 1920. Serial No. 359,507.

To all whom it may concern:

Be it known that we, JAMES A. SINGMASTER and FRANK G. BREYER, both citizens of the United States, residing at Palmerton, Carbon County, State of Pennsylvania, have invented certain new and useful Improvements in Production of Zinc Oxide; and we do hereby declare the following to be a full, clear, and exact description of the invention, such as will enable others skilled in the art to which it appertains to make and use the same.

This invention relates to improvements in the Wetherill process for the production of zinc oxide, free or relatively free from lead, from high grade zinciferous material such as oxidized ores, roasted or semi-roasted sulfide ores, or calcined carbonate ores, etc., which ores are rich in zinc and relatively low in gangue.

By the Wetherill process as referred to herein, we mean the furnacing step of the process for producing zinc oxide in which a charge of the zinciferous material mixed with a reducing agent and spread on an ignited bed of fuel is subjected to a combustion supporting blast or draft and brought to a sufficiently high temperature to reduce the compounds of zinc and volatilize the reduced metal, without bringing the charge to a condition where it becomes impervious to the blast or draft; the entire charge being supported on a furnace hearth or grate designed to hold it without letting any considerable part drop through, and the worked-off material being discharged as a clinker or sinter.

In the commercial production of zinc oxide by means of the Wetherill process, it has heretofore been customary to first charge upon the perforated hearth or grate of the furnace a layer of "buckwheat" anthracite coal (which is thereupon ignited by the residual heat of the furnace) and, by means of a forced draft, to bring this initial layer of coal to well developed combustion. Upon this layer of "bed coal" or "ignition coal" is then charged the customary mixture or "working charge" characteristic of the Wetherill process, that is to say, a mixture of finely-divided reducing coal with the finely-divided zinciferous material. The forced air draft is continued, and, when the familiar flames of greenish tint, known as

"zinc candles" begin to make their appearance above the upper surface of the charge, indicating that the reduction and volatilization of the zinc and its oxidation to the form of fume is well under way, the products of combustion carrying the zinc oxide fume and other volatilized metallic compounds are conveyed through the customary cooling flues, etc., to the bag-room wherein, in a cooled condition, they filter through the bags and pass off into the atmosphere, leaving the fume collected in the interior of the bags, from which it is removed at convenient intervals. The furnace operation is continued until the production of fume therefrom in appreciable quantity ceases, whereupon the residual charge, which is, to a large extent, sintered together, is broken up by long handled rabbles and pried up and lifted or scraped out through the furnace doors into a receiving pit, or the like, preparatory to the starting of a new operation.

The Wetherill process is fundamentally a sintering process, as distinguished from smelting processes in which fusion and scoriafication takes place. In the Wetherill process no fusion and no scoriafication is permissible, or is permissible only to a slight degree, such as will result in the formation of a clinker sufficiently porous to permit the air blast to pass therethrough. If fusion takes place and the slag thus formed runs down on the grate, the grate becomes clogged and the operation of the process is thereby prevented.

The zinciferous materials heretofore commonly used in the production of zinc oxide by the Wetherill process have been relatively low grade materials, such as low grade zinc ores, relatively high in gangue and clinker-forming constituents, while high grade zinciferous material, such as ores rich in zinc, have been commonly used for the production of spelter or metallic zinc. With low grade ores, having a relatively low zinc content and a large amount of gangue, a relatively thick layer of admixed ore and coal can be used in the working charge, and this thick layer can be distributed over the grate in the form of a relatively thick layer of approximately uniform thickness, which will assist in the uniform distribution of the air through the grate and through the charge, and which will offer a sufficient and suf-

ficiently uniform resistance to the air blast to permit the process to be continued to substantial completion.

- If an attempt is made to use an amount of high grade ore comparable to the amount of low grade ore commonly used, together with the necessary coal for its proper treatment, it is found that the gangue constituents in the lower portion of the charge, 5 after the working off of the zinc oxide and the combustion of the carbonaceous material therefrom, tend to fuse together and form an impervious layer of slag or clinker immediately above the grate, thus interfering 10 with the uniform action of the blast, and resulting in uneven working of the charge, or even in the prevention of the further carrying on of the process. As a result, the tendency to the formation of cracks or of blow- 15 holes or craters at various regions of the charge is increased, and it becomes difficult to maintain a uniform working off of the charge, while a considerable amount of the zinc of the upper portions of the charge re- 20 mains in the residue. The zinc contained in these residues cannot ordinarily be recovered commercially, and is therefore lost.

These objections to the use of such a thick working charge of high grade ore can be 25 decreased by reducing the thickness of the working charge. With such a thin working charge, however, a lower blast pressure must be employed, while the difficulty of maintaining a uniform distribution of the blast is 30 greatly increased, and difficulty is still met with from the tendency towards formation of an impervious layer of slag or clinker immediately above the grate.

- These difficulties in the working of high grade zinciferous material can, by the process of the present invention, be overcome or obviated to such an extent that it becomes possible to employ, in the Wetherill process, 40 a working charge containing high grade zinciferous material, comparable in thickness and amount to the charges of low grade zinciferous material heretofore commonly employed, so that very materially increased yields or makes can be obtained per square foot of grate area.

The process of the present invention, therefore, relates to the treatment of such high grade zinciferous material, such as oxidized ores, roasted or semi-roasted 45 sulfide ores, or calcined carbonate ores etc., which are relatively rich in zinc and free from or low in lead, so that there will be obtained a zinc oxide which is free or relatively free from lead, and containing, for example, not more than three percent of lead, figured as lead sulfate, and preferably less than one percent; that is, the process of the invention relates to the production of a high grade zinc oxide of low lead content, as distinguished from products of relatively high

lead content, commonly known as leaded zinc oxide.

We have discovered that if a layer of slate coal is spread uniformly over the layer of ignition coal, after it has been brought to a well developed combustion, and if the working charge is then charged into the furnace and spread out upon the layer of slate coal, the thickness of the working charge containing the high grade zinciferous material can be increased to a thickness comparable with the thickness of the working charge of low grade zinciferous materials heretofore commonly employed, and the requisite porosity of the charge can be thereby maintained throughout the working off operation, and a sufficiently increased pressure of the air blast can be used, so that the charge can be worked off to substantial completion, with the result that very materially increased recoveries can be obtained from the heavier burdens thus employed, that is, very materially increased recoveries of high grade zinc oxide can be thus obtained from furnaces of the same grate area heretofore employed in the production of very materially less amounts of zinc oxide. High grade zinciferous material of the character above referred to; such as oxidized ores, roasted sulfide ores or concentrates or calcined carbonate ores or 50 concentrates, etc. such as have heretofore been commonly used in the manufacture of spelter, can, according to the present invention, be advantageously employed in the manufacture of zinc oxide. Ores or concentrates, for example, flotation concentrates, can thus be employed, which, after roasting, contain from 50 to 70 per cent or more of zinc, that is, of very materially higher zinc content than the low grade ores, containing 55 for example, 30 per cent or less of zinc, such as have commonly heretofore been employed in the practice of the Wetherill process.

We have also discovered that the treatment of such high grade ores can be further improved by admixing slate coal with the working charge, so that there is both a layer of the slate coal between the firing coal or ignition coal and the working charge, and further amounts of slate coal 110 admixed with the working charge itself. The layer of slate coal thus employed contributes to the process by the combustion of its contained coal and by providing a porous distributing layer between the ignition coal and the working charge, while the slate coal admixed with the working charge contributes in a similar manner to the maintenance of the charge in a sufficient state of porosity for the satisfactory carrying out of the Wetherill process. Even though the gangue constituents of the high grade ore may tend to fuse and form a slag, this slag will be prevented from matting together and forming a layer which will close 115 120 125 130

the grate. The slate coal itself is substantially non-slagging and retains its form until the carbonaceous portion thereof has been removed; while whatever sintering takes place thereafter does not interfere with the proper working of the charge. Accordingly, a sufficient air blast can be forced through the charge and with sufficient uniformity, so that, as above noted, the working charge can be worked off to substantial completion, with resulting high recovery and increased production from the high grade ore employed.

The nature and advantages of the invention, and the invention itself, will be further illustrated from the following specific example, showing comparative results obtained by the practice of the invention, and by the practice of the Wetherill process without a layer of slate coal between the firing coal and the charge or slate coal mixed with the charge. A representative analysis of the ore employed is as follows:

|    |                        |        |  |
|----|------------------------|--------|--|
| 25 | ZnO-----               | 69.00% |  |
|    | PbO-----               | 0.15%  |  |
|    | S-----                 | 5.00%  |  |
|    | SiO <sub>2</sub> ----- | 2.5%   |  |
| 30 | FeO-----               | 13.0%  |  |
|    | CaO-----               | 2.5%   |  |

Two furnace blocks were worked with the ore. The charge for each charge door, that is, one-third of the charge for each furnace, in each case, was as follows:

|                           |          |          |  |
|---------------------------|----------|----------|--|
| Roasted sulfid ore-----   | 690 lbs. | 690 lbs. |  |
| Coal in charge-----       | 920 lbs. | 920 lbs. |  |
| Slate coal in charge----- | 250 lbs. | -----    |  |
| 40 Firing coal-----       | 250 lbs. | 250 lbs. |  |
| Slate on firing coal----- | 200 lbs. | -----    |  |

In the operating of the respective furnaces, it was found that the amount of the air blast on the furnaces which were operated without slate coal (used in the manner above described) could only be increased very slightly beyond the initial amount, and that, in attempting to increase the amount of the air blast, the charge would break from the grate, thus preventing the continuation of the process. With the furnaces operating with the charges in which the slate coal was used (in the manner above described) it was found possible to increase the air blast gradually until the full air blast had been attained at about one hour before drawing the fire. It was thus found possible to use an average of about 40 per cent more air with the furnaces in which the slate coal was employed (in the manner above described) as compared with the furnaces where the slate coal was not employed.

The amount of clinker obtained and the zinc oxide and carbon content thereof, are

given below. The amounts given are from a charge three times that above given, that is, from one furnace, while the charge above given is for each charge door, or for one third of the furnace.

|                                        |           |           |    |    |
|----------------------------------------|-----------|-----------|----|----|
| Wgt. of clinker from 1<br>furnace----- | 2355 lbs. | 1355 lbs. |    | 70 |
| Percent ZnO in clinker-----            | 4.6%      | 12.2%     |    |    |
| Percent C in clinker-----              | 16.9%     | 21.9%     |    |    |
| ZnO lost in clinker-----               | 8.92%     | 13.61%    |    |    |
| Percent of ZnO charged-----            |           |           | 75 |    |

It will be noted that a much greater loss of zinc oxide took place where the slate coal was not employed (in the manner above described) than when it was so employed; while the weight of the clinker obtained when the slate coal was employed is very materially increased in amount, owing to the slate content of the slate coal so used.

The bag-room recoveries obtained in each case showed a recovery of about 71 per cent over a period of several days, as compared with an average recovery of more than 84 percent from the furnaces where the slate coal was employed.

The low recovery of 71% is too low for commercial operations. In order to increase the recovery (when slate coal is not employed) to above 80% it is necessary to reduce the burden of the high grade ore to such an extent that the yields are not materially greater than with low grade ores, e. g., around 9500 lbs. zinc oxide per 24 hours from one block (of four furnaces). Where slate coal is employed (in the manner above described) with high grade ore, it is possible to increase the yield to around 16,500 lbs. per 24 hours or even higher, from the same grate area, while still obtaining high recoveries, such as above referred to.

Instead of employing slate coal in the manner above described, other materials may be employed which are substantially non-slagging and which serve to provide a porous distributing layer between the ignition coal and the working charge. Slate alone or bone coal may thus be employed, as well as other materials of a suitable character. The material should be of a suitable size, preferably between about one half inch and one inch. The material which we consider most advantageous, however, is slate coal, preferably the portion rejected in the preparation of anthracite coal by jigging, inasmuch as it contributes combustible material to the process, as well as a substantially non-slagging material, and inasmuch as the presence of the coal intimately admixed with the slate improves the action of the slate for the purposes of the invention. Accordingly we recommend slate coal as the material to be used when it is available inasmuch as it is a waste product commonly

found in large amounts wherever coal is mined, it is readily obtainable in large amount and at moderate expense. Where bituminous shales of suitable character are available, these can be used in a similar manner.

The layer of slate coal (or other material) can be employed alone, without admixture of further amounts of slate coal with the working charge, and we consider this to be a characteristic feature of the invention, irrespective of whether further amounts of the slate coal are employed in the working charge. However, it will usually be more advantageous to supply further amounts of the slate coal to the working charge, so that there will be obtained both the advantages of the layer of slate coal between the layer of ignition coal and the working charge, and the advantages of the slate coal admixed with the working charge itself.

The single figure of the accompanying drawing diagrammatically represents the invention as carried out in a furnace of the Wetherill type. As indicated in the drawing, the furnace has a flat horizontal grate composed of heavy cast iron sections with slot perforations to permit of the passage of air through them. Beneath the grate are ash pits 2 where the material falling through the grate accumulates and is removed from time to time through suitable ash-pit doors 3. The furnace is commonly constructed of fire brick within and red brick without and provided with the usual stays and supports (not shown). The capacity of the furnace is determined by the area of the grate. This grate may, for example, have a length of about 19½ feet and a width of about 6 feet, the top of the arch 4 being about 3 feet above the top of the grate. The furnace has a plurality of charge doors 5 through which the various constituents of the charge are spread upon the grate after being dumped down through suitable holes 6 in the top of the furnace provided for this purpose. The fume-laden gases are conducted from the furnace through upright pipes 7 which communicate in the well understood manner with a suitable bag-house for collecting zinc oxide. As indicated by the legends on the accompanying drawing, a layer of non-slaggering material is charged into the furnace between the layer of ignition fuel and the working charge, the latter containing high grade zinciferous material with or without admixture of further amounts of non-slaggering material.

What we claim is:

1. In the production of zinc oxide by the Wetherill process from a working charge containing high grade zinciferous material relatively low in gangue constituents, the step of supplying a porous distributing layer

of substantially non-slaggering material between the ignition fuel and the working charge; substantially as described.

2. In the production of zinc oxide by the Wetherill process from a working charge containing high grade zinciferous material relatively low in gangue constituents, the step of supplying a porous distributing layer of substantially non-slaggering material between the ignition fuel and the working charge, together with the step of adding further amounts of such material in admixture with the working charge; substantially as described.

3. In the production of zinc oxide by the Wetherill process from a working charge containing high grade roasted or semi-roasted sulfide ores or concentrates or calcined carbonate ores or concentrates, the step of supplying a porous distributing layer of substantially non-slaggering material between the ignition fuel and the working charge; substantially as described.

4. In the production of zinc oxide by the Wetherill process from a working charge containing high grade roasted or semi-roasted sulfide ores or concentrates or calcined carbonate ores or concentrates, the step of supplying a porous distributing layer of substantially non-slaggering material between the ignition fuel and the working charge, together with the step of adding further amounts of such material in admixture with the working charge; substantially as described.

5. In the production of zinc oxide by the Wetherill process from a working charge containing high grade zinciferous material relatively low in gangue constituents, the step of supplying a layer of slate coal between the ignition fuel and the working charge; substantially as described.

6. In the production of zinc oxide by the Wetherill process from a working charge containing high grade zinciferous material relatively low in gangue constituents, the step of supplying a layer of slate coal between the ignition fuel and the working charge, together with the step of supplying further amounts of slate coal in admixture with the working charge; substantially as described.

7. In the production of zinc oxide by the Wetherill process from a working charge containing high grade roasted or semi-roasted sulfide ores or concentrates or calcined carbonate ores or concentrates, the step of supplying a layer of slate coal between the ignition fuel and the working charge; substantially as described.

8. In the production of zinc oxide by the Wetherill process from a working charge containing high grade roasted or semi-roasted sulfide ores or concentrates or calcined

carbōnate ores or concentrates, the step of supplying a layer of slate coal between the ignition fuel and the working charge, together with the step of supplying further amounts of slate coal in admixture with the working charge; substantially as described.

9. The method of smelting volatilizable metals of the nature of lead or zinc particularly applicable to practice with a great furnace which comprises providing a bed

of refractory particles, supporting thereon a charge of mixed metalliferous material and reduction fuel and supplying air to the charge through the bed to support combustion whereby even penetration of the charge and emission of the metal as vapor are assured. 15

In testimony whereof we affix our signatures.

JAMES A. SINGMASTER.  
FRANK G. BREYER.

**Certificate of Correction.**

It is hereby certified that in Letters Patent No. 1,450,704, granted April 3, 1923, upon the application of James A. Singmaster and Frank G. Breyer, of Palmerton, Pennsylvania, for an improvement in "Production of Zinc Oxide," errors appear in the printed specification requiring correction as follows: Page 1, line 80, for the word "takes" read *take*; page 2, line 21, for the misspelled word "beemes" read *becomes*, and line 73, after the word "coal" strike out the period and insert a comma; page 3, line 26, for "PfO" read *PfO*, and line 75, for "ZnoO" read *ZnO*; page 5, line 10, claim 9, for the word "great" read *grate*; and that the said Letters Patent should be read with these corrections therein that the same may conform to the record of the case in the Patent Office.

Signed and sealed this 5th day of June, A. D., 1923.

KARL FENNING,  
*Acting Commissioner of Patents.*

[SEAL]